# EUROPEAN PATENT SPECIFICATION

(11) **EP 3 486 925 B1**
(45) Date of publication and mention of the grant of the patent: **09.09.2020**
(21) Application number: 18206278.6
(22) Date of filing: 14.11.2018
(51) Int. Cl.: H01F 1/057, H01F 7/02, H01F 41/02, C25D 3/12, C25D 3/22, C25D 3/38, C25D 3/56, C25D 5/12, C25D 7/00

(54) **NDFEB MAGNET WITH COMPOSITE COATING AND PREPARATION PROCESS THEREOF**
NDFEB-MAGNET MIT VERBUNDSTOFFBESCHICHTUNG UND HERSTELLUNGSVERFAHREN DAFÜR
AIMANT NDFEB À REVÊTEMENT COMPOSITE ET SON PROCÉDÉ DE PRÉPARATION

(30) Priority: 17.11.2017 CN 201711141628
(43) Date of publication of application: 22.05.2019
(73) Proprietor: Yantai Shougang Magnetic Materials Inc., 265500 Yantai (CN)
(72) Inventor: Xie, Changbo, Yantai City, 265500 (CN); Chen, Dejin, Yantai City, 265500 (CN)
(74) Representative: Gulde & Partner

(56) References cited:
- CN-A- 104 099 648
- CN-A- 106 968 003
- CN-A- 109 137 022
- CN-B- 103 898 505

## Description

The invention relates to the technical field of surface treatment of neodymium iron boron magnets, in particular to a neodymium iron boron magnet with composite coating and a preparation process thereof.

### Technical Background

The newly developed NdFeB magnet is a third-generation rare earth material, usually composed of a main phase of Nd₂Fe₁₄B and a neodymium-rich phase at the grain boundary. It is a magnetic functional material with poor corrosion resistance and magnetic structure susceptible to temperature. In order to address said problem, specific coatings have been developed.

Currently, surface coatings of NdFeB magnets include electroplated layers or layer stacks, such as a Zn layer, a Ni-Ni layer, a Ni-Cu-Ni layer, and an Al layer, or an epoxy layer, each having benefits and disadvantages. In particular, thermal demagnetization of magnets with a Ni-Ni layer or a Ni-Cu-Ni layer, especially of small sized products such as mobile components, is inappropriate. Further, the wear resistance of a Zn layer, an Al layer or an epoxy layer is poor. When the products require both wear resistance and low thermal demagnetization, the present coatings are insufficient to satisfy both requirements at the same time.

CN 106 968 003 A discloses an NdFeB magnet coated by Zn/ZnNi/Ni/Cu/Ni, without specifying a thickness or the Ni content in the NiZn layer.

### Summary of Invention

It is an object of the present invention to overcome the deficiencies of the prior art and, in particular, to provide a neodymium iron boron magnet having a superior composite coating.

Another object of the present invention is to provide a process for preparing a neodymium iron boron magnet having a composite plating layer.

The invention should also solve or at least lessen the problem that the prior nickel-plating process of the neodymium-iron-boron magnet has a great influence on the thermal demagnetization of the magnet and the relative adhesion to the substrate.

According to an aspect of the present invention there is provided a NdFeB magnet with a composite coating disposed on an outer surface of the NdFeB magnet as defined in claim 1.The composite coating comprises or consists of:
- a zinc layer (directly) disposed on the surface of the NdFeB magnet, wherein a thickness of the zinc layer is 0.1-10µm;
- a zinc-nickel alloy layer (directly) disposed on the zinc layer, wherein a thickness of the zinc-nickel alloy layer is 0.1-10µm and a content of nickel within the zinc-nickel alloy is 5-25 wt.%;
- a copper layer (directly) disposed on the zinc-nickel alloy layer, wherein a thickness of the copper layer is 0.1-10µm; and
- a nickel layer covering (directly) disposed on the copper layer, wherein a thickness of the nickel layer is 0.1-10µm.

In other words, the technical solution of the present invention is a neodymium iron boron magnet comprising a neodymium iron boron base body, which is special in that the neodymium iron boron base body has a composite plating layer structure. The composite plating layer structure includes a galvanized zinc layer, a galvanized zinc-nickel alloy layer, a copper plating layer and finally a nickel plating layer. The thickness of the galvanized zinc layer is 0.1-10 microns, the thickness of the zinc-nickel alloy layer is 0.1-10 microns, and the nickel content in the zinc-nickel alloy layer is 5-25 wt.%, the thickness of the copper plating layer is 0.1- 10 microns; and the electroplated nickel layer thickness is 0.1-10 microns.

According to another aspect of the present invention there is provided a preparation process of the before mentioned composite coated NdFeB magnet. The process includes the steps as defined in claim 2.

In particular, there is provided a process of preparing a composite coating on an outer surface of an NdFeB magnet, the process including the steps of:
a) optionally, grinding chamfer: the NdFeB magnet body is ground and chamfered by centrifugal or vibrating finishing machine for 1-10 hours;
b) optionally, degreasing: using hot dip degreasing solution to remove oil stain on the surface of the magnet body;
c) optionally, cleaning: thoroughly wash the surface of the magnet body with water;
d) optionally, pickling: using a nitric acid with a mass fraction of 1-10% to clean rust and oxide layers on the surface of the magnet body;
e) optionally, ultrasonic cleaning: Using ultrasonic equipment to thoroughly clean the ash on the surface of the magnet body;
f) optionally, activation: lightly corrode the surface of the magnet body with an acid at a volume concentration of 0.1-1%;
g) optionally, cleaning: thoroughly clean the surface of the magnet body with tap water and pure water respectively;
h) electroplating zinc: electroplating a layer of zinc on the magnet body using a zinc plating solution until a thickness of the plating layer is 0.1-10 µm;
i) optionally, cleaning: washing the surface of the magnet body with nitric acid having a volume concentration of 0.1-3%;
j) electroplating zinc-nickel alloy: electroplating a zinc-nickel alloy layer on the surface of the zinc layer using a zinc-nickel alloy plating solution until a thickness of the zinc-nickel alloy layer is 0.1-10 µm, wherein the nickel content in the plating layer is 5-25%;
k) optionally, cleaning: the surface of the magnet body is thoroughly washed with water;
l) electroplating copper: electroplating a copper layer on the surface of the zinc-nickel alloy layer using a copper plating solution until a thickness of the plating layer is 0.1-10 µm;
m) optionally, activation: lightly corrode the surface of the copper layer with hydrochloric acid in a volume concentration of 1-5%, and then thoroughly clean the surface of the substrate with water;
n) electroplating nickel: electroplating a nickel layer on the surface of the copper layer using a nickel plating solution until a thickness of the plating layer is 0.1-10 µm; and
o) optionally, cleaning and drying: the magnet body is washed with tap water and pure water, respectively, and then dried.

Preferably, at least one of the electroplating steps h), l), j), and n) is performed by using a rack or barrel plating method.

The inventive composite coating possesses excellent corrosion resistance and the influence of coating on thermal demagnetization of magnets is extremely small on the surface of NdFeB magnet. A composite coating with complete compactness and uniform brightness can be obtained. The composite coating has little influence on the performance of the magnet, which greatly reduces the thermal demagnetization rate of the magnet. The bonding strength between the coating and the substrate is firm and can meet the cross-cutting, thermal vibration, drop, push-pull force test requirements. The composite coating shows excellent corrosion resistance, specifically a neutral salt spray test can reach 96 hours. Further, the process control is simple and easy to promote.

Preferably, the zinc electroplating solution contains 20-120g/L ZnCl, 120-320g/L KCl, 10-100g/L H₃BO₃, 0.1-50g/L additives (e.g. zinc acid additive, like HT-MB zinc acid additive, and zinc acid brightener), and the pH of the electroplating solution is 3.0-6.0.

Preferably, the zinc-nickel alloy electroplating solution contains 2-20g/L Zn²⁺, 1-10g/L Ni²⁺, 50-200g/L metal ion complexing agent and 20-200g/L NaOH.

Preferably, the copper electroplating solution contains 20-120g/L cupric pyrophosphate, 100-300g/L potassium pyrophosphate, 0.1-50g/L additives (e.g. brightener and a PL coke copper cylinder opening agent), and the pH of the electroplating solution is 7.0-10.0.

Preferably, the nickel electroplating solution contains 150-350g/L NiSO₄, 10-100g/L NiCl₂, 10-100g/L H₃BO₃, 0.1-50g/L additives (e.g. nickel brightener, such as Ni-88, and softener, such as A-5), and the pH of the electroplating solution is 3.0-5.0.

The NdFeB magnet with composite plating and the preparation process thereof have outstanding substantive features and significant progress compared with the prior art: 1. The composite coating has almost no influence on the thermal demagnetization rate of the magnet; The bonding strength between the composite coating and the substrate is very good; 3. The corrosion resistance of the composite coating is greatly improved.

### Detail Description the Invention

The invention is described in detail below with reference to the embodiments of the invention, and is not intended to limit the scope of the invention.

The invention relates to a neodymium iron boron magnet with composite coating and a preparation process thereof. The basic principle is that a neodymium iron boron substrate is immersed in a solution of a metal salt as a cathode, and a metal plated is used as an anode. A metal plating layer is deposited on the substrate of the cathode.

### Example 1

The embodiment illustrates the specific technology of NdFeB magnet plating by using barrel plating. The matrix is ground and chamfered to that R is 0.2-0.3mm, and the duration of grinding and chamfering is 3 hours. The oil impurity of matrix surface is cleaned with hot dipped deoiling solution that volume concentration is 40g/L, and the surface of matrix is cleaned with spray water for 1-2min. The next, the oxidation layer and the corrosion layer are cleaned with nitric acid solution that mass fraction is 3% for 60s. The dust on the surface of matrix is thoroughly cleaned by ultrasonic equipment for 3min, and then the surface of matrix is softly corroded with nitric acid solution that mass fraction is 1%. After pickling and ultrasonic cleaning, the matrix is thoroughly cleaned by tap water and pure water for 60s, respectively. The processed samples are loaded into the six corner drum and then plated in the zinc electroplating solution composed of 20-120g/L ZnCI, 120-320g/L KCI, 10-100g/L H₃BO₃, 0.1-50g/L HT-MB zinc acid additive and zinc acid brightener, and the pH of the electroplating solution is adjusted to 3.0-6.0. The size of drum is determined by the size of matrix, and the thickness of plating layer is limited to 0.1-10µm. After zinc plating, the samples are polished homogeneously with dilute nitric acid that volume concentration is 1%, and then cleaned by tap water and pure water for 60s, respectively. After the last process, the samples are plated in zinc-nickel alloy electroplating solution composed of 2-20g/L Zn²⁺, 1-10g/L Ni²⁺, 50-200g/L metal ion complexing agent and 20-200g/L NaOH. The thickness of plating layer is limited to 0.1-10µm and the content of nickel is 5-25% in the plating layer. Next, the samples are cleaned by water, and then plated in copper electroplating solution composed of 20-120g/L cupric pyrophosphate, 100-300g/L potassium pyrophosphate, 0.1-50g/L PL coke copper cylinder opening agent and brightener, and the pH of the electroplating solution is adjusted to 7.0-10.0. In order to avoid the replacement reaction in electroplating process, the samples can be electrified before immersed into the electrolyzer. The thickness of copper plating layer is limited to 0.1-10µm. After copper plating, the samples are activated in hydrochloric acid or sulphuric acid that volume concentration is 3%, and then cleaned by water. Next, the samples are plated in nickel electroplating solution composed of 150-350g/L NiSO₄, 10-100g/L NiCl₂, 10-100g/L H₃BO₃, 0.1-50g/L Ni-88 brightener and A-5 softener. The pH of electroplating is adjusted to 3.0-5.0 and the thickness of electroplating is limited 0.1-10µm. After nickel electroplating, the samples are washed by water as well as dried in centrifuge or dried by blower. The structure of composite coating is zinc+ zinc-nickel alloy+ copper+ nickel.

The size of the product is 9.14*6.39*0.85mm and the name of the product is 48H. A salt spray test of the plated product showed that the size does not change for at least 96 hours. At 120°C, the thermal demagnetization of the product is less than 2%. Through thrust test, the maximum thrust that coating can bear is greater than 300N.

In a comparative test, a product of the same size was plated with a Ni-Cu-Ni coating. Rust appeared after salt spray test for 72 hours. At 120°C, the average thermal demagnetization of product plated Ni-Cu-Ni coating was 8%. Through thrust test, the average maximum thrust that Ni-Cu-Ni coating can bear was 220N.

### Example 2

In the second embodiment, a product with a large sized magnet is plated by track plating. The matrix is ground and chamfered to that R is 0.4-0.5mm, and the duration of grinding chamfering is 10 hours. After chamfering, the oil impurity of matrix surface is cleaned with hot dipped deoiling solution having a volume concentration of 40g/L, and the surface of matrix is cleaned with spray water for 1-2min. Next, the oxidation film and the corrosion film are cleaned with nitric acid solution that mass fraction is 1-10% for 90s. The dust on the surface of matrix is thoroughly cleaned by ultrasonic equipment for 5min, and then the surface of matrix is softly corroded for 30s with nitric acid solution that volume concentration is 0.1-1%. After pickling and ultrasonic cleaning, the matrix is thoroughly cleaned by tap water and pure water for 60s, respectively. The processed samples are loaded into a six corner drum and then plated in the zinc electroplating solution composed of 20-120g/L ZnCI, 120-320g/L KCI, 10-100g/L H₃BO₃, 0.1-50g/L HT-MB zinc acid additive and zinc acid brightener, and the pH of the electroplating solution is 3.0-6.0. The size of drum is determined by the size of matrix, and the thickness of layer is limited to 0.1-10µm. After zinc plating, the samples are polished homogeneously with dilute nitric acid that volume concentration is 0.1-3%, and then cleaned by water. After the last process, the samples are plated in zinc-nickel alloy electroplating solution composed of 2-20g/L Zn²⁺, 1-10g/L Ni²⁺, 50-200g/L metal ion complexing agent and 20-200g/L NaOH. The thickness of the layer is limited to 0.1-10µm and the content of nickel is 5-25% in the layer. Next, the samples are cleaned by water, and then plated in copper electroplating solution composed of 20-120g/L cupric pyrophosphate, 100-300g/L potassium pyrophosphate, 0.1-50g/L PL coke copper cylinder opening agent and brightener, and the pH of the electroplating solution is adjusted to 7.0-10.0. The thickness of coating is limited to 0.1-10µm. After copper electroplating, the surface of matrix is activated by sulfuric acid and hydrochloric acid that volume concentration is 1-5% for 60s, and then the matrix is cleaned by water. Next, the samples are plated in nickel plating solution composed of 150-350g/L NiSO₄, 10-100g/L NiCl₂, 10-100g/L H₃BO₃, 0.1-50g/L Ni-88 brightener and A-5 softener. The pH of the plating solution is adjusted to 3.0-5.0 and the thickness is limited to 0.1-10µm. After nickel electroplating, the samples are washed by water as well as dried in centrifuge or dried by blower. The structure of composite coating is zinc+ zinc-nickel alloy+ copper+ nickel.

### Example 3

The process is similar to Example 1 except the following differences. The duration of grinding and chamfering is 10 hours. The oxidation film and the corrosion film on the surface are cleaned by acid for 30s. The dust on the surface is thoroughly cleaned by ultrasonic equipment for 1min. The duration of samples are activated by nitric acid that volume concentration is 0.1-10% is 5s, and then samples are cleaned by tap water and pure water for 60s. After copper plating, the samples are activated by sulfuric acid and hydrochloric acid that volume concentration is 1-5% for 10s.

The inventive NdFeB magnets possess a composite coating that layer structure is "Zn+ Zn-Ni alloy+ Cu+ Ni". The NdFeB magnets are plated with a film of zinc layer after grinding chamfering, oil removal, pickling, ultrasonic clean and activation. The combination of zinc coating and the matrix is extreme strong and the zinc coating can not affect the thermal reduction rate of magnets. On the basic zinc coating and as transition layers, the zinc-nickel alloy layer and the copper layer are plated on the surface of the samples. It ensures that the adhesion of each coating is strong while the corrosion resistance of the coating is greatly improved. Finally, a film of nickel layer is plated on the copper layer to make whole plating coating stable, wearable, and possessing excellent adhesion and corrosion resistance.

## Claims

1. An NdFeB magnet with a composite coating disposed on an outer surface of the NdFeB magnet, the composite coating comprising or consisting of:
- a zinc layer disposed on the surface of the NdFeB magnet, wherein a thickness of the zinc layer is 0.1-10µm;
- a zinc-nickel alloy layer disposed on the zinc layer, wherein a thickness of the zinc-nickel alloy layer is 0.1-10µm and a content of nickel within the zinc-nickel alloy is 5-25 wt.%;
- a copper layer disposed on the zinc-nickel alloy layer, wherein a thickness of the copper layer is 0.1-10µm; and
- a nickel layer covering disposed on the copper layer, wherein a thickness of the nickel layer is 0.1-10µm.

2. A process for preparing a composite coating on an outer surface of an NdFeB magnet, the process including the steps of:
a) optionally, grinding chamfer: the NdFeB magnet body is ground and chamfered by centrifugal or vibrating finishing machine for 1-10 hours;
b) optionally, degreasing: using hot dip degreasing solution to remove oil stain on the surface of the magnet body;
c) optionally, cleaning: thoroughly wash the surface of the magnet body with water;
d) optionally, pickling: using a nitric acid with a mass fraction of 1-10% to clean rust and oxide layers on the surface of the magnet body;
e) optionally, ultrasonic cleaning: Using ultrasonic equipment to thoroughly clean the ash on the surface of the magnet body;
f) optionally, activation: lightly corrode the surface of the magnet body with an acid at a volume concentration of 0.1-1%;
g) optionally, cleaning: thoroughly clean the surface of the magnet body with tap water and pure water respectively;
h) electroplating zinc: electroplating a layer of zinc on the magnet body using a zinc plating solution until a thickness of the plating layer is 0.1-10 µm;
i) optionally, cleaning: washing the surface of the magnet body with nitric acid having a volume concentration of 0.1-3%;
j) electroplating zinc-nickel alloy: electroplating a zinc-nickel alloy layer on the surface of the zinc layer using a zinc-nickel alloy plating solution until a thickness of the zinc-nickel alloy layer is 0.1-10 µm, wherein the nickel content in the plating layer is 5-25%;
k) optionally, cleaning: the surface of the magnet body is thoroughly washed with water;
l) electroplating copper: electroplating a copper layer on the surface of the zinc-nickel alloy layer using a copper plating solution until a thickness of the plating layer is 0.1-10 µm;
m) optionally, activation: lightly corrode the surface of the copper layer with hydrochloric acid in a volume concentration of 1-5%, and then thoroughly clean the surface of the substrate with water;
n) electroplating nickel: electroplating a nickel layer on the surface of the copper layer using a nickel plating solution until a thickness of the plating layer is 0.1-10 µm; and
o) optionally, cleaning and drying: the magnet body is washed with tap water and pure water, respectively, and then dried.

3. The process of claim 2, wherein the zinc plating solution contains 20-120g/L ZnCI, 120-320g/L KCI, 10-100g/L H₃BO₃, 0.1-50g/L additives, and the pH of the plating solution is adjusted to 3.0-6.0.

4. The process of claim 2, wherein the zinc-nickel alloy plating solution contains 2-20g/L Zn²⁺, 1-10g/L Ni²⁺, 50-200g/L metal ion complexing agent and 20-200g/L NaOH.

5. The process of claim 2, wherein the copper electroplating solution contains 20-120g/L cupric pyrophosphate, 100-300g/L potassium pyrophosphate, 0.1-50g/L additives, and the pH of the electroplating solution is adjusted to 7.0-10.0.

6. The process of claim 2, wherein the nickel electroplating solution contains 150-350g/L NiSO₄, 10-100g/L NiCl₂, 10-100g/L H₃BO₃, 0.1-50g/L additives, and the pH of the electroplating solution is adjusted to 3.0-5.0.

## Patentansprüche

1. NdFeB-Magnet mit einer Verbundstoffbeschichtung, die auf einer Außenfläche des NdFeB-Magneten angeordnet ist, wobei die Verbundstoffbeschichtung Folgendes umfasst oder daraus besteht:
- eine(r) Zinkschicht, die auf der Oberfläche des NdFeB-Magneten angeordnet ist, wobei eine Dicke der Zinkschicht 0,1 - 10 µm beträgt;
- eine(r) Zink-Nickel-Legierungsschicht, die auf der Zinkschicht angeordnet ist, wobei eine Dicke der Zink-Nickel-Legierungsschicht 0,1 - 10 µm beträgt und ein Nickelgehalt innerhalb der Zink-Nickel-Legierung 5 - 25 Gew.-% beträgt;
- eine(r) Kupferschicht, die auf der Zink-Nickel-Legierungsschicht angeordnet ist, wobei eine Dicke der Kupferschicht 0,1 - 10 µm beträgt; und
- eine(r) Nickelschichtabdeckung, die auf der Kupferschicht angeordnet ist, wobei eine Dicke der Nickelschicht 0,1 - 10 µm beträgt.

2. Verfahren zur Herstellung einer Verbundstoffbeschichtung auf einer Außenfläche eines NdFeB-Magneten, wobei das Verfahren folgende Schritte umfasst:
a) optional Schleifen einer Abschrägung: der NdFeB-Magnetkörper wird mit einer Zentrifugal- oder Vibrations-Endbearbeitungsmaschine 1-10 Stunden lang geschliffen und abgeschrägt;
b) optional Entfetten: unter Benutzung einer heißen Eintauch-Entfettungslösung, um Ölflecken auf der Oberfläche des Magnetkörpers zu entfernen;
c) optional Reinigen: gründliches Waschen der Oberfläche des Magnetkörpers mit Wasser;
d) optional Beizen: unter Benutzung einer Salpetersäure mit einer Massenfraktion von 1 - 10 %, um die Oberfläche des Magnetkörpers von Rost und Oxidschichten zu reinigen;
e) optional Ultraschallreinigen: unter Benutzung von Ultraschalltechnik, um die Oberfläche des Magnetkörpers gründlich von der Asche zu reinigen;
f) optional Aktivierung: leichtes Korrodieren der Oberfläche des Magnetkörpers mit einer Säure mit einer Volumenkonzentration von 0,1 - 1 %;
g) optional Reinigen: gründliches Reinigen der Oberfläche des Magnetkörpers, entsprechend mit Leitungswasser und reinem Wasser;
h) galvanisches Verzinken: galvanisches Abscheiden einer Zinkschicht auf dem Magnetkörper unter Benutzung eines Verzinkungsbades, bis eine Dicke der Überzugsschicht 0,1 - 10 µm beträgt;
i) optional Reinigen: Waschen der Oberfläche des Magnetkörpers mit Salpetersäure mit einer Volumenkonzentration von 0,1 - 3 %;
j) galvanisches Überziehen mit einer Zink-NickelLegierung: galvanisches Abscheiden einer Zink-Nickel-Legierungsschicht auf der Oberfläche der Zinkschicht unter Benutzung eines Zink-Nickel-Legierungs-Galvanisierungsbades, bis eine Dicke der Zink-Nickel-Legierungsschicht 0,1 - 10 µm beträgt, wobei der Nickelgehalt in der Überzugsschicht 5 - 25 % beträgt;
k) optional Reinigen: die Oberfläche des Magnetkörpers wird gründlich mit Wasser gewaschen;
l) galvanisches Verkupfern: galvanisches Abscheiden einer Kupferschicht auf der Oberfläche der Zink-Nickel-Legierungsschicht unter Benutzung eines Verkupferungsbades, bis eine Dicke der Überzugsschicht 0,1 - 10 µm beträgt;
m) optional Aktivierung: leichtes Korrodieren der Oberfläche der Kupferschicht mit Chlorwasserstoffsäure mit einer Volumenkonzentration von 1 - 5 % und dann gründliches Reinigen der Oberfläche des Substrats mit Wasser;
n) galvanisches Vernickeln: galvanisches Abscheiden einer Nickelschicht auf der Oberfläche der Kupferschicht unter Benutzung eines Vernickelungsbades, bis eine Dicke der Überzugsschicht 0,1 - 10 µm beträgt; und
o) optional Reinigen und Trocknen: der Magnetkörper wird entsprechend mit Leitungswasser und reinem Wasser gewaschen und dann getrocknet.

3. Verfahren nach Anspruch 2, wobei das Verzinkungsbad 20 - 120 g/l ZnCl, 120 - 320 g/l KCl, 10 - 100 g/l H₃BO₃ und 0,1 - 50 g/l Additive enthält und der pH-Wert des Galvanisierungsbades auf 3,0 - 6,0 eingestellt wird.

4. Verfahren nach Anspruch 2, wobei das Zink-Nickel-Legierungs-Galvanisierungsbad 2 - 20 g/l Zn²⁺, 1 - 10 g/l Ni²⁺, 50 - 200 g/l Metallionen-Komplexbildner und 20 - 200 g/l NaOH enthält.

5. Verfahren nach Anspruch 2, wobei das Verkupferungsbad 20 - 120 g/l Kupferpyrophosphat, 100 - 300 g/l Kaliumpyrophosphat und 0,1 - 50 g/l Additive enthält und der pH-Wert des Galvanisierungsbades auf 7,0 - 10,0 eingestellt wird.

6. Verfahren nach Anspruch 2, wobei das Vernickelungsbad 150 - 350 g/l NiSO₄, 10 - 100 g/l NiCl₂, 10 - 100 g/l H₃BO₃ und 0,1 - 50 g/l Additive enthält und der pH-Wert des Galvanisierungsbades auf 3,0 - 5,0 eingestellt wird.

## Revendications

1. Aimant de type NdFeB à revêtement composite disposé sur une surface externe de l'élément de type NdFeB, le revêtement composite comprenant ou étant constitué :
- d'une couche de zinc disposée sur la surface de l'élément de type NdFeB, dans lequel une épaisseur de la couche de zinc est comprise entre 0,1 et 10 µm ;
- d'une couche d'alliage de zinc et de nickel disposée sur la couche de zinc, dans lequel une épaisseur de la couche d'alliage de zinc et de nickel est comprise entre 0,1 et 10 µm et une teneur en nickel à l'intérieur de l'alliage de zinc et de nickel est comprise entre 5 et 25 % en poids ;
- d'une couche de cuivre disposée sur la couche d'alliage de zinc et de nickel, dans lequel une épaisseur de la couche de cuivre est comprise entre 0,1 et 10 µm ; et
- d'un revêtement de couche de nickel disposé sur la couche de cuivre, dans lequel une épaisseur de la couche de nickel est comprise entre 0,1 et 10 µm.

2. Procédé de préparation d'un revêtement sur une surface externe d'un aimant de type NdFeB, le procédé comprenant les étapes de :
a) éventuellement, chanfrein de meulage : le corps d'aimant de type NdFeB est broyé et chanfreiné au moyen d'une machine de finition centrifuge ou vibrante pendant une durée allant de 1 à 10 heures ;
b) éventuellement, dégraissage : utilisation d'une solution de dégraissage de trempage à chaud afin d'éliminer les taches d'huile sur la surface du corps d'aimant ;
c) éventuellement, nettoyage : laver soigneusement la surface du corps d'aimant avec de l'eau ;
d) éventuellement, décapage : utilisation d'un acide nitrique ayant une fraction massique comprise entre 1 et 10 % afin de nettoyer la rouille et les couches d'oxydation sur la surface du corps d'aimant ;
e) éventuellement, nettoyage par ultrasons : utilisation d'un équipement ultrasonique pour nettoyer soigneusement les cendres sur la surface du corps d'aimant ;
f) éventuellement, activation : corroder légèrement la surface du corps d'aimant avec un acide ayant une concentration volumique comprise entre 0,1 et 1 % ;
g) éventuellement, nettoyage : nettoyer soigneusement la surface du corps d'aimant avec de l'eau du robinet et avec de l'eau pure respectivement ;
h) galvanoplastie sur zinc : électroplacage d'une couche de zinc sur le corps d'aimant au moyen d'une solution de placage de zinc jusqu'à ce qu'une épaisseur de la couche de placage soit comprise entre 0,1 et 10 µm ;
i) éventuellement, nettoyage : lavage de la surface du corps d'aimant avec de l'acide nitrique ayant une concentration volumique comprise entre 0,1 et 3 % ;
j) électroplacage d'un alliage de zinc et de nickel : électroplacage d'une couche d'alliage de zinc et de nickel sur la surface de la couche de zinc en utilisant une solution de placage d'alliage de zinc et de nickel jusqu'à ce qu'une épaisseur de la couche d'alliage de zinc et de nickel soit comprise entre 0,1 et 10 µm, dans lequel la teneur en nickel dans la couche de placage est comprise entre 5 et 25 % ;
k) éventuellement, nettoyage : la surface du corps d'aimant est lavée soigneusement avec de l'eau ;
l) galvanoplastie sur cuivre : électroplacage d'une couche de cuivre sur la surface de la couche d'alliage de zinc et de nickel en utilisant une solution de placage de cuivre jusqu'à ce qu'une épaisseur de la couche de placage soit comprise entre 0,1 et 10 µm ;
m) éventuellement, activation : corroder légèrement la surface de la couche de cuivre avec de l'acide chlorhydrique ayant une concentration volumique comprise entre 1 et 5 %, et ensuite laver soigneusement la surface du substrat avec de l'eau ;
n) galvanoplastie sur nickel : électroplacage d'une couche de nickel sur la surface de la couche de cuivre en utilisant une solution de placage de nickel jusqu'à ce qu'une épaisseur de la couche de placage soit comprise entre 0,1 et 10 µm ; et
o) éventuellement, nettoyage et séchage : le corps d'aimant est lavé avec de l'eau du robinet et de l'eau pure, respectivement, et est ensuite séché.

3. Procédé selon la revendication 2, dans lequel la solution de placage de zinc contient de 20 à 120 g/L de ZnCl, de 120 à 320 g/L de KCl, de 10 à 100 g/L de H₃BO₃, de 0,1 à 50 g/L d'additifs, et le pH de la solution de placage est ajusté pour être compris entre 3,0 et 6,0.

4. Procédé selon la revendication 2, dans lequel la solution de placage d'alliage de zinc et de nickel contient de 2 à 20 g/L de Zn²⁺, de 1 à 10 g/L de Ni²⁺, de 50 à 200 g/L d'un agent de complexion d'ions métalliques et de 20 à 200 g/L de NaOH.

5. Procédé selon la revendication 2, dans lequel la solution d'électroplacage de cuivre contient de 20 à 120 g/L de pyrophosphate cuprique, de 100 à 300 g/L de pyrophosphate de potassium, de 0,1 à 50 g/L d'additifs, et le pH de la solution d'électroplacage est ajusté pour être compris entre 7,0 et 10,0.

6. Procédé selon la revendication 2, dans lequel la solution d'électroplacage de nickel contient de 150 à 350 g/L de NiSO₄, de 10 à 100 g/L de NiCl₂, de 10 à 100 g/L de H₃BO₃, de 0,1 à 50 g/L d'additifs, et le pH de la solution de placage est ajusté pour être compris entre 3,0 et 5,0.
